

# UNITED STATES PATENT OFFICE.

WILLIAM WARBURTON, OF STOCKPORT, ENGLAND.

## COMPOSITION OF MATTER FOR USE IN EXTRACTING VEGETABLE FIBERS.

SPECIFICATION forming part of Letters Patent No. 634,154, dated October 3, 1899.

Application filed June 1, 1897. Serial No. 638,938. (No specimens.)

*To all whom it may concern:*

Be it known that I, WILLIAM WARBURTON, a subject of the Queen of Great Britain and Ireland, and a resident of 70 Adswood Lane, 5 East, Stockport, county of Chester, England, have invented a certain new Composition of Matter for Use in Extracting Vegetable Fibers, of which the following is a specification.

My said invention relates to a new composition of matter treating the various fibrous plants of the nettle family commonly known as "ramie," "rhea," "china-grass," or other similar fibrous vegetable products for the purpose of extracting fibers therefrom. Acids of 15 various kinds have been used heretofore for such a purpose; but in practice they are found to reduce the strength and to otherwise damage the fibers.

I subject such fibrous material to the action 20 of an emulsion or solution containing carbonate of soda in combination with soap and petroleum and bicarbonate of soda (or an equivalent quantity of carbonate of ammonia) in a closed vessel or keir under steam-pressure.

I prefer to treat the vegetable material in the form of ribbons, such as are usually found in commerce. These are for convenience of handling laid in baskets of galvanized wire, 30 which are then placed in an ordinary high-pressure keir, such as is commonly found in bleach-works. Sufficient water is run into the keir to cover the material. Meanwhile in a separate receptacle I prepare a liquid 35 mixture as follows: For every hundred parts, by weight, of fibrous material to be treated I usually take seventeen parts of "pure alkali," seven parts of soap, eleven parts of petroleum, ten parts of bicarbonate of soda. These are

40 mixed with water in the proportion of three hundred parts, by weight, to form a solution, emulsion, or mixture which will readily flow into the keir. By pure alkali I mean the form of sodium carbonate ( $Na_2CO_3$ ) known 45 commercially under that name and which contains about fifty-eight per cent. of sodium oxid, ( $Na_2O$ .) For the bicarbonate of soda ( $NaHCO_3$ ) an equal weight of commercial carbonate of ammonia, which ordinarily consists

50 chiefly of  $NH_4HCO_3$  with  $NH_4NH_2CO_2$  and a

trace of  $(NH_4)_2CO_3$ , may be substituted. This mixture is run into the keir containing the submerged fibrous material, whereupon the keir is closed, steam is admitted, and the whole is kept under steam-pressure for a suitable time, depending to some extent on the nature or kind of material being treated. For the ordinary ramie ribbons of commerce I find that if it is subjected to the action of the above-described mixture under a steam-pressure of fifty to fifty-five pounds per square inch for four to five hours it is sufficient. The proportions of pure alkali and bicarbonate of soda are subject to variation, according to the nature and origin of the material 55 to be treated. Some materials require more or less pure alkali, (with a corresponding diminution or augmentation of the bicarbonate of soda.) For example, in treating ramie grown on a limestone soil I should use ten 60 parts only of pure alkali and seventeen parts of bicarbonate of soda, (or of carbonate of ammonia.) The proportions of soap and petroleum remain practically the same in any case. After such treatment it will be found 70 that the gummy or resinous constituents of the fibrous material and also the skin are dissolved, decomposed, or altered in such a way that subsequent washing with pure water suffices to eliminate them from the fiber. This 75 subsequent washing may be accomplished by hand or with the aid of machinery or mechanical appliances of various kinds, as will be well understood by those conversant with the treatment of fibrous materials without further description.

What I claim as my invention, and desire to secure by Letters Patent, is—

A composition of matter for use in extracting vegetable matters and consisting of pure 90 alkali, soap, petroleum and bicarbonate of soda substantially as defined and in the proportions set forth.

In testimony whereof I have signed my name to this specification in the presence of 95 two subscribing witnesses.

WILLIAM WARBURTON.

Witnesses:

JOHN HALL,  
A. T. WHITELOW.